

## UNITED STATES PATENT OFFICE.

ANTHONY PEPPER, OF PATERSON, NEW JERSEY.

## PROCESS FOR WEIGHTING SILKS.

No Drawing.

Application filed August 14, 1925. Serial No. 50,271.

*To all whom it may concern:*

Be it known that I, ANTHONY PEPPER, a citizen of the United States, and a resident of Paterson, in the county of Passaic and 5 State of New Jersey, have invented certain new and useful Improvements in Processes for Weighting Silks, of which the following is a specification.

This invention relates to a process for 10 weighting silks by means of chemical compounds.

In the production of silk fabrics it is necessary to treat the silks before dyeing with a chemical which will give sufficient 15 weight to the fabric and which will not be objectionable because of its effect upon the skin of a wearer. It is well known that the halogen compounds of tin have been employed for the purpose but due to the fact 20 that it is difficult to obtain a stannic compound free of impurities such compounds have therefore been very unsatisfactory. Lead acetate has also been suggested but is also considered objectionable due to the fact 25 that when the silk containing such acetate comes in contact with the skin it will cause irritation.

It is an object of the present invention to 30 provide a process in which a compound of tin and of lead may be employed for weighting the silk which will have none of the objectionable features ordinarily found and in which the materials after being treated 35 with stannic chloride are then treated to a solution of sodium phosphate. After washing the goods thus treated are at a pre-determined temperature placed in a weak solution of acetic acid. A solution of lead acetate is then applied and after washing 40 the materials are placed in a cold solution of sodium phosphate.

A further object of the invention is the 45 provision of a process in which silk fabrics are treated with a compound of tin after which the goods are placed in a solution of sodium phosphate at a predetermined temperature for approximately one hour. After 50 the goods have been washed they are treated with a warm and weak solution of acetic acid and after washing they are successively treated with a lead acetate solution and cold sodium phosphate solution.

This invention will be best understood 55 from a consideration of the following de-

tailed description; nevertheless it is to be understood that the invention is not confined to the disclosure, being susceptible of such changes and modifications which shall define no material departure from the salient features of the invention as expressed in the appended claims.

In carrying out my invention a solution of stannic chloride  $\text{SnCl}_4$  at 20° Baumé is prepared and the silk fabrics are placed in the solution for approximately one hour and 60 after such time they are removed and washed in order to remove the excess halogen compound.

After the washing process the fabrics are placed in a solution of sodium phosphate 70 of 7° Baumé and at a temperature of 150° F. where the fabrics are permitted to remain for approximately one hour when they are removed and washed in clear water. The steps in the above noted process are repeated 75 approximately three times.

After the last washing the fabrics are then placed in a 3% solution of acetic acid and at a temperature of 160° F. The fabrics are allowed to remain in this solution for approximately one-half hour when they are treated with cold water and are then placed in a lead acetate solution at 150° F. and permitted to remain there for one hour. The lead acetate is the normal or diacetate of 80 lead known as sugar of lead and having an empirical formula  $\text{Pb}(\text{C}_2\text{H}_3\text{O}_2)_2$ . The temperature of the acetate solution is maintained at 150° F. and the solution is approximately of 2 to 3 degrees Baumé. The 85 fabrics are permitted to remain in the solution for one hour after which they are washed. They are then placed in a cold sodium phosphate solution for one-half hour when they are removed and dried and then 90 are ready for dyeing.

By the treatment of the stannic chloride and the treatment of the lead acetate with sodium phosphate injurious effects of the lead acetate have been neutralized so that 100 the goods thus treated do not have the objectionable features as if they were simply treated by the stannic chloride and by the lead acetate. In either case the sodium phosphate tends to neutralize the acid reaction of the stannic chloride and also that of the sugar of lead and it is possible that 105 some of the acetate of lead is converted into

tribasic lead phosphate  $Pb_3(PO_4)_2$ . The tribasic phosphate salt of lead may be formed when a small quantity of sodium phosphate is added to an excess of lead acetate.

The step in the process by which the silk fabrics are treated with stannic chloride and sodium phosphate with the number of necessary washings is the usual method for 10 preliminarily treating silk fabrics before dyeing. When the fabrics are treated with a weak solution of acetic acid and the lead acetate the fabrics absorb a predetermined quantity of the lead acetate so that when 15 the sodium phosphate is placed in solution and the fabrics are treated an insoluble salt of lead is formed which will not be acted upon by the perspiration and thereby affect the skin of the wearer.

20 What I claim is:

1. A process for weighting silk fabrics which comprises placing the fabrics in a solution of stannic chloride of 20° Baumé for approximately one hour, then washing the 25 fabrics, treating the washed fabrics with a solution of sodium phosphate of 7° Baumé at a temperature of 150° F. for approximately one hour, then washing the fabrics, treating the washed fabrics with a 3% solution of acetic acid at 160° F. for one half hour, washing the fabric with cold water, treating the fabric with a solution of lead acetate of approximately 3° Baumé at a 30 temperature of 150° F. for one hour and 35 then after washing treating the fabrics with a cold solution of sodium phosphate for one half hour.

2. A process for weighting silk fabrics which comprises placing the fabric in a 40 solution of stannic chloride for one hour then washing the fabric, treating the washed fabric with a solution of sodium phosphate for approximately one hour, then washing the fabric, treating the washed fabrics with a weak solution of acetic acid for approximately one half hour, washing the fabric with cold water, treating the fabric with a 45 solution of lead acetate for approximately one hour, and then washing said fabric and 50 treating the same with a cold solution of

sodium phosphate for approximately one-half hour.

3. A process for weighting silk fabrics which comprises treating the fabrics with a solution of stannic chloride, then washing 55 the fabrics, treating the washed fabrics with a solution of sodium phosphate, then washing the fabrics, treating the washed fabrics with a solution of acetic acid, then washing the fabrics with cold water, treating the 60 fabrics with a solution of lead acetate, then washing the fabrics and treating the same with a cold solution of sodium phosphate.

4. A step in the process for weighting silk fabrics which comprises treating silk 65 fabrics with a weak solution of acetic acid for approximately one half hour, washing the fabrics thus treated in cold water, then treating the washed fabrics with a solution of lead acetate for approximately one hour, 70 washing said fabrics, and then treating said fabrics with a cold solution of sodium phosphate for approximately one half hour.

5. A step in the process for weighting silk fabrics which comprises treating silk 75 fabrics with a hot solution of acetic acid for approximately one-half hour, washing said fabrics in cold water and then treating the fabrics with a hot solution of lead acetate of approximately 3° Baumé for approximately 80 one hour, then washing the fabric and treating the same with a cold solution of sodium phosphate for approximately one half hour.

6. A step in the process for weighting silk fabrics which comprises treating silk 85 fabrics with a weak solution of acetic acid, washing the fabrics thus treated in cold water, then treating the washed fabrics with a solution of lead acetate, washing said fabrics, and then treating said fabrics with a cold solution of sodium phosphate.

7. A step in the process for weighting silk fabrics which comprises treating silk 90 fabrics with a weak solution of acetic acid, treating the fabrics with a solution of lead acetate, and then treating the fabrics with a solution of sodium phosphate.

ANTHONY PEPPER.